

# UNITED STATES PATENT OFFICE.

FOSTER MILLIKEN, OF LAWRENCE, NEW YORK.

## ALLOY.

1,310,363.

Specification of Letters Patent. Patented July 15, 1919.

No Drawing.

Application filed August 29, 1918. Serial No. 251,942.

*To all whom it may concern:*

Be it known that I, FOSTER MILLIKEN, a citizen of the United States, and a resident of Lawrence, county of Nassau, and State of New York, have invented a new and Improved Alloy, of which the following is a full, clear, and exact description.

This alloy differs from the alloy covered by my Patent No. 1,277,989 in that the quantity of iron present therein is higher in proportion than that which has been disclosed in the above-mentioned patent.

This alloy is characterized by its resisting qualities at high temperature, which renders the said alloy more suitable for molds for molten glass. It is further characterized by the ease with which it can be machined, and therefore it renders the formation of the molds comparatively inexpensive. The al-

loy contains the following metals in substantially the following proportions:

|        |       |           |
|--------|-------|-----------|
| Copper | 56-64 | per cent. |
| Nickel | 13-17 | " "       |
| Zinc   | 10-15 | " "       |
| Iron   | 10-15 | " " 25    |

These metals are melted together and cast in the usual way and the alloy resulting therefrom possesses a peculiar non-oxidizing quality. It is of the necessary density, has good machining qualities and effectively radiates heat, thereby adapting the metal for work where high temperatures are present.

I claim:

An alloy formed from 56-64 per cent. copper, 13-17 per cent. nickel, 10-15 per cent. zinc, and 10-15 per cent. iron.

FOSTER MILLIKEN.